

Aug. 1, 1950

M. ARDITI ET AL

2,516,841

GRID FOR ELECTRON DISCHARGE DEVICES

Filed Jan. 16, 1946

4 Sheets-Sheet 1



Fig. 1.



Fig. 2.



INVENTORS  
MAURICE ARDITI  
VINCENT J. DESANTIS  
BY

R. P. Morris  
ATTORNEY

Aug. 1, 1950

M. ARDITI ET AL

2,516,841

GRID FOR ELECTRON DISCHARGE DEVICES

Filed Jan. 16, 1946

4 Sheets-Sheet 2

Fig. 4.



INVENTORS  
MAURICE ARDITI  
VINCENT J. DE SANTIS  
BY

*R.P. Morris*  
ATTORNEY

Aug. 1, 1950

M. ARDITI ET AL

2,516,841

GRID FOR ELECTRON DISCHARGE DEVICES

Filed Jan. 16, 1946

4 Sheets-Sheet 3



PLATE VOLTAGE

INVENTORS  
MAURICE ARDITI  
VINCENT J. DE SANTIS

BY

*R. Morris*  
ATTORNEY

Aug. 1, 1950

M. ARDITI ET AL

2,516,841

GRID FOR ELECTRON DISCHARGE DEVICES

Filed Jan. 16, 1946

4 Sheets-Sheet 4



INVENTORS  
MAURICE ARDITI  
VINCENT J. DESANTIS  
BY

R.P. Morris  
ATTORNEY

Patented Aug. 1, 1950

2,516,841

# UNITED STATES PATENT OFFICE

2,516,841

## GRID FOR ELECTRON DISCHARGE DEVICES

Maurice Ardit, New York, N. Y., and Vincent J. De Santis, Chatham, N. J., assignors to Federal Telephone and Radio Corporation, New York, N. Y., a corporation of Delaware

Application January 16, 1946, Serial No. 641,580

3 Claims. (Cl. 250—177)

1

2

This invention relates to grids for electron discharge devices. The grid core metal is preferably molybdenum or tungsten or any workable high melting metal which will not sag or warp at red or even white ultra-high and micro-wave frequencies usually operating temperatures. Molybdenum is a metal which dissipates disproportionately large amounts of heat energy. The grid is heated by induction, because of its malleability. The surface of the core by electron and ion bombardment, and by radiation from the cathode, and because of the fine wire construction of the grid, the grid is first of carbide of boron (B<sub>6</sub>C). Finely powdered boron carbide is made to adhere to the core to reach the limiting temperature of the tube. Even at temperatures below which the grid normally operates, there may be considerable primary emission from the wires and a consequent shortening of the tube input impedance. Finally, gas is evolved and metals evaporated from the grid to give an even, smooth non-porous and some-what carbonized appearance to the grid. One suitable grain-size for use is found to be 800 mesh. One will poison and reduce cathode emission.

An object of this invention is improved grids for electron discharge devices. Electron discharge devices having a grid with a boron carbide surface have been found to operate throughout a normal life at rated power levels, with low grid emission, and normal cathode emission. Good results were obtained with low primary and secondary emission, low vapor pressure, and good electrical conductivity.

A more specific object of this invention is a grid of metal having a high melting point, and a surface with black body characteristics, having a low primary and secondary emission, low vapor pressure, and good electrical conductivity.

The characteristic features of this invention are defined in the appended claims, and a preferred embodiment is described in the following specification and shown in the accompanying drawings, in which:

Fig. 1 is a vertical sectional view of one electron discharge device having the novel grid of this invention;

Fig. 2 is a typical grid structure;

Fig. 3 is a section of the novel grid; and

Figs. 4, 5 and 6 are curves showing comparative operational characteristics of grids treated according to our invention.

The discharge device of Fig. 1 is of the medium power, high-frequency type in which the grid is subject to considerable heating. The anode 1, cathode 2 and grid 3 are cylindrical and coaxial and are sealed in envelope 4, the lead-in for the anode being sealed at the lower end of the envelope, well removed from the grid and cathode supports 5 and 6 respectively. The desirable properties of the novel grid here described are obtained when the cathode is the conventional, barium-strontium oxide coated core. One simple grid structure shown in Fig. 2 comprises an upper central supporting member 7 and a spaced supporting band or collar 8 to which are secured by spot welding a plurality of fine vertical grid wires 9. A spiral of fine wire 10 is wound around the cylinder formed by wires 9 and secured to the wires, for example, by welding to make the structure rigid.

The above-described grid was made by spraying a wet mixture of the powdered boron carbide

on the wires of a prefabricated grid structure.

One specific mixture found to give good results was prepared by ball milling commercial boron carbide.

An inert liquid binder and vehicle for the powder consisting of 26 cc. of pyroxolin or

nitrocellulose dissolved in 243 cc. of amyl acetate was used, sufficient powder being mixed in the liquid to produce a paint of such a consistency as to spray well from an air-operated spray gun.

Uniform coatings on the grids were obtained by mounting the grids in rotating fixtures and alternately spraying and drying with infra-red radiation.

The passes were repeated until about 10 milligrams of coating per square centimeter were deposited, whereupon the coating was baked under

an infra-red light. The coated grids were then

ium fired to degas the grid and to firmly ad-  
the coating to the core. When heated to  
degrees centigrade in vacuum, boron car-  
appears to form a sintered layer at the  
rface of the carbide powder and the core. The  
grid is black and smooth in appearance,  
lar to a carbonized surface.

another grid coating which was also satis-  
sory was prepared as follows:

to 25 cc. of tetraethyl orthosilicate is added  
cc. of material composed mainly of ethyl alco-  
denatured with methyl alcohol, ethyl acetate,  
yl isolintylketane and aviation gasoline.  
added material is commercially available  
er the trade name of "Synasol." This mix-  
is stirred until it is uniform. Then to this  
ure is added 5 cc. of .3% hydrochloric acid  
the solution is stirred until hydrolysis is com-  
ed and allowed to stand three hours before  
27 grams of boron carbide (800 mesh) are  
into a mortar and 40.5 cc. of the binder mix-  
described above is put in at the rate of about  
cc. at a time. Between each addition of the  
er the mixture is ground with a pestle until  
orm, care being taken to see that the final  
ure is free of all lumps.

1 grids to be coated with this mixture should  
be vapor degreased in trichloroethylene and  
heated in an atmosphere of hydrogen at  
degrees C. for fifteen minutes. When these  
ations are complete the grids are not touched

bare hands. The prepared boron carbide  
ure is then sprayed on the surface of the  
using as fine a spray as possible. In order  
cilitate the deposition of a smooth uniform  
ing, the grids should be rotated at about 100  
M. during application of the coating. Suf-  
t coating should be sprayed onto the surface  
sure complete coverage. It was found that  
it 3 milligrams per square centimeter of  
ed surface is the optimum weight of coating.  
ter the grid has been sprayed the coating  
be dried by placing it about four inches  
an infra-red radiating lamp, the grid being  
ly turned. The coated grid may then be  
bled in the tube. If desired the grids may  
rst vacuum fired before they are assembled  
e final tube.

ie vacuum firing may be carried out in the  
ope in which the grid is finally mounted  
the other electrodes, or the firing may be  
in a separate envelope or bell-jar before  
nly, high frequency induction being the  
practical source of heating energy.  
urning now to Fig. 4, the operating character-  
s of the tube prepared in accordance with  
invention may be observed. This figure  
s grid emission in microamperes plotted in  
mi-logarithmic scale against the grid power  
t in watts. Curves 11 and 12 illustrate the  
emission obtained from pure molybdenum  
; after twenty one and thirty two hours  
ation respectively, while curves 13 and 14  
grid emission curves on the same scale for  
treated with boron carbides. This shows  
grid emission is reduced to an extremely  
value while the untreated grids have ex-  
ely high emission.

urning now to Fig. 5, a comparison is shown  
een the cathode emission and plate voltage  
ubes having treated and untreated grids. In  
ntreated grids as shown in curves 15, 16 and  
filament voltages of 7, 6.3 and 6 volts respec-  
y, are shown. At 18, 19 and 20 are shown  
similar respective curves for the cathode

emission in tubes having the treated grids. It  
is seen that the cathode emission is higher for  
these tubes with the treated grids than it is for  
the tubes using the untreated grids, again the  
filament voltages being 7, 6.3 and 6 respectively.

In Fig. 6 is shown curve 21 illustrating the  
grid emission in milliamperes plotted against  
grid input in watts for a tube having a tungsten  
carbide treated grid. Curve 22 shows a similar  
10 grid emission curve in a common standard in  
low grid emission, that is, a gold plated grid.  
Curves 23 and 24 illustrate boron carbide treated  
15 grids, curve 24 showing the operation after age-  
ing for one hundred and forty hours. For all  
20 grid inputs the boron carbide grids are shown  
to be far superior to the tungsten carbide treated  
grids. For all grid inputs above ten the boron  
carbide grid is shown to be superior to the gold  
plated grid. Furthermore, after one hundred and  
25 forty hours of ageing with a power input to the  
cathode as high as 25 watts the grid emission  
from the boron carbide treated grid is even lower  
than it was initially as clearly demonstrated in  
curve 24.

25 The grid of this invention will emit negligible  
quantities of electrons even at high operating  
temperatures and will not adversely affect  
cathode emission. The grid has good conduc-  
30 tivity for high frequency current and is simple  
and easy to manufacture.

We claim:

35 1. An electron discharge device comprising a  
cathode having an emissive coating of mixed  
oxides of barium and strontium, and a control  
electrode, said control electrode comprising a  
core of molybdenum bearing an adherent, external  
coating of a mixture of boron carbide and  
an inert binder on said core.

40 2. An electron discharge device comprising a  
cathode having an emissive coating of mixed  
oxides of barium and strontium, and a control  
electrode, said control electrode comprising a  
core of molybdenum, a layer of sintered par-  
45 ticles of boron carbide and the core material on  
said core, and a layer of a mixture of boron car-  
bide and an inert binder on said layer of sintered  
particles.

50 3. An electron discharge device comprising a  
cathode having an emitting surface of barium-  
strontium oxides and a control electrode, said  
control electrode comprising a core of molyb-  
denum, a layer of sintered particles of boron car-  
55 bide and the core material on said core, and a  
smooth, external layer of a mixture of boron car-  
bide and an inert binder on said layer of sintered  
particles.

MAURICE ARDITI.  
VINCENT J. DE SANTIS.

#### REFERENCES CITED

The following references are of record in the  
file of this patent:

#### UNITED STATES PATENTS

| Number    | Name       | Date          |
|-----------|------------|---------------|
| 1,934,477 | Barton     | Nov. 7, 1933  |
| 2,164,699 | Clark      | July 4, 1939  |
| 2,232,083 | Strohfeldt | Feb. 18, 1941 |
| 2,417,730 | Becker     | Mar. 18, 1947 |

#### FOREIGN PATENTS

| Number  | Country     | Date          |
|---------|-------------|---------------|
| 209,022 | Switzerland | June 1, 1940  |
| 217,145 | Switzerland | Jan. 16, 1942 |